

## UNITED STATES PATENT OFFICE

TREADWAY B. MUNROE, OF CHICAGO, ILLINOIS, ASSIGNOR TO THE CELOTEX COMPANY,  
OF CHICAGO, ILLINOIS, A CORPORATION OF DELAWARE

## METHOD OF DRYING

No Drawing.

Application filed April 5, 1930. Serial No. 442,035.

This invention relates to a method for drying fibrous materials, particularly to the drying of such materials after formation thereof into board-like sheets formed on a machine generally similar to machines employed in the formation of paper, and has for its object to provide a method which is more efficient in operation than those heretofore proposed.

10 The material to be dried, according to the method disclosed herein, is more particularly the board-like materials which are now made and sold as insulating building boards, substantially all of which are made 15 from vegetative or wood fiber. In the manufacture of boards of this type the raw material is not reduced to a condition suitable for the manufacture of paper, but instead the reduction is to fiber bundles comprising 20 a plurality of fibers, although incidental to such reduction there is, of course, some reduction of the material to elemental fibers.

In the drying of these fibrous materials, after they have been sheeted on a board 25 machine from a dilute suspension thereof, the conditions are in general quite different from the conditions met in drying paper sheets. That is, it is possible to express 30 the suspending fluid from the sheeted stock down to a point at which there is substantially no free fluid therein and, due to the fact that the fibers are hydrated but very slightly if at all, there is little or no water 35 of hydration to be removed from the sheeted stock.

In the ordinary drying of paper stock there are generally considered to be three 40 stages of water removal;—first, the evaporation of what might be termed the loosely held water, that is the water mechanically held in the sheet in the larger fiber interstices; second, the removal of the water which is retained in the sheet due to capillarity;—and the third stage comprising the

removal of the chemically or physically combined water of hydration.

It has been determined that a sheeted insulating board formed from sugar cane bagasse fiber bundles has characteristics which 50 make it particularly adaptable to the new method of drying which will hereinafter be more fully described. In addition to the use of this method in connection with the drying of insulating board made from sugar 55 cane bagasse, the method may be advantageously employed in the drying of other fibrous insulating boards such as those made from wood, straw, corn stalks, and the like although, for various reasons which will be 60 evident, the results will not be quite as satisfactory as are obtained in the drying of board made from sugar cane bagasse.

In the manufacture of these insulating boards the raw material, whether sugar cane 65 bagasse, wood, corn stalks, straw, or the like, is lightly digested or otherwise prepared for separation into fiber bundles, which separation is accomplished preferably by means of swing hammer shredders or 70 equivalent refining machines. Due to the fact that in the initial preparation of the fibrous materials there is, in general, substantially nothing removed therefrom except the water soluble materials, such fiber 75 bundles retain a considerable amount of lignin and various inorganic constituents, and in the case of bagasse and straw there is particularly an appreciable content of complex silica compounds. The lignin content and these inorganic compounds tend 80 to make the fibers relatively stiff whereby, when compressed, they generally tend to return to their original condition, which feature is available to some extent in the 85 described method of drying.

After the fibers are sheeted from their dilute suspension in a machine of the nature of a paper-making machine, the sheets pass through squeeze rolls, which remove from 90

the sheet substantially all of the loosely retained water, or at least as much thereof as can be removed without crushing the sheet.

The freshly formed sheet is passed from the press rolls into a tunnel drier of a type generally well-known to those engaged in the industry and such for example as illustrated in U. S. Letters Patent No. 1,501,966 granted July 22, 1924 to Treadway B. Munro and wherein, by the passage of heated unsaturated gas over the surfaces of the board, water is removed therefrom.

It has been discovered that, by the removal of substantially all of the loosely contained water from the formed sheet through the use of the press rolls, the subsequent drying of the sheet in a tunnel drier comprises drying at a continuously decreasing rate of water removal and that, due to the fact that these sheets are approximately one-half inch thick, as the sheets are dried the exterior portions thereof serve as non-conductors thereby greatly retarding the removal of moisture from the interior of the sheet.

It has been determined that, for instance, one-half of the residual moisture may be removed from the sheet in the tunnel drier in approximately the same time as is required for the removal of the succeeding quarter of the original moisture, and that the removal of the next one-eighth of the residual moisture requires about the same time as does the removal of the first half of the moisture content.

By subjecting all surfaces of the sheet in a tunnel drier to heat sufficient to remove about one-half of the moisture content which it contained on entering the drier, and then completing the drying in a press having heated platens, such as is shown in U. S. Letters Patent No. 984,870 granted Feb. 21, 1911 to J. A. Wheeler it has been discovered that the drying may be carried out more rapidly and more economically. It has been found that by placing the sheets between heated platens having provision such as interposed screens or the like for the escape of such steam as may be formed in the course of drying, a more rapid heat transfer may be obtained into the interior of the sheet, since by applying pressure to the heated platens, the board being dried can be somewhat compacted, whereby the rate of heat transfer is improved, and further, the heat transfer is improved, due to the intimate contact of the heated platens with the opposed surfaces of the board being dried.

In the drying of insulating boards according to the method just described it has been found, particularly in the drying of insulating boards made from sugar cane bagasse if the boards are initially dried in the tunnel drier to approximately 20% moisture content, that appreciable pressure can be

placed thereon by the platens of the press, whereby the final rate of drying may be increased and the time of drying decreased, but that due to the resiliency of the fibers because of the relatively high lignin content and residual inorganic matter, when the pressure is released, the board tends to return to its original dimensions, and this is substantially true of insulating boards made from corn stalk fiber, straw, wood fiber, and the like, although for certain of these materials the tendency of the sheet to return to its original dimensions after release of the pressure is less than that of sheets made from sugar cane bagasse.

It is obvious that those skilled in the art may vary the steps and combinations of steps constituting this method within the scope of this invention without departing from the spirit thereof, and therefore it is not desired to be limited to the foregoing disclosure except as may be demanded by the claims.

What is claimed is:

1. The method of drying board composed primarily of fiber bundles unsuitable for paper-making and fiber, wherein after formation of the sheet from dilute water suspension, with subsequent removal of its loosely held water, the sheet is dried in a tunnel drier to not less than 20% moisture content and subsequently fully dried between heated press platens while subjected to compression therebetween.

2. The method of drying fiber insulating board comprising the initial extraction of water therefrom in a tunnel drier to a moisture content of not less than 20% with subsequent drying while subjected to compression between heated press platens.

3. The method of drying insulating board made from fiber bundles derived from sugar cane bagasse, straw, wood, and the like, wherein sheeted fiber bundles thereof formed from a dilute water suspension are first subjected to pressure between squeeze rolls for the removal of the loosely held water therein, are subsequently subjected to a current of heated unsaturated gaseous medium for the removal of approximately one-half of its moisture content, and finally are subjected to compression between heated press platens for the complete removal of the moisture content thereof.

4. The method of manufacturing a board-like product composed of fiber bundles and fiber, wherein the final stage of manufacture comprises serial drying initially to a moisture content of not less than 20% by vapor circulation, and finally through subjection to pressure between heated press platens and the like.

5. The method of drying freshly formed fiber board comprising the initial extraction of water therefrom to a moisture content of

70

75

80

85

90

95

100

105

110

115

120

125

130

not less than 20% by contact with a heated gas, and the final drying thereof while subjected to pressure between heated surfaces.

6. The method of drying freshly formed fiber board comprising the initial extraction of water therefrom by contact of all surfaces with a heated gas, and the final drying thereof by contact of opposed surfaces with heated members while subjected to pressure therebetween.

In testimony whereof I affix my signature.

TREADWAY B. MUNROE.

15

20

25

30

35

40

45

50

55

60

65